

June 5, 1928.

1,672,631

E. A. TROEGER

TRANSLUCENT SCREEN FOR PROJECTION MACHINES

Filed Aug. 21, 1925



Inventor  
Ernest A. Troeger.

By his Attorneys  
Cooper, Kerr & Dunham

## UNITED STATES PATENT OFFICE.

ERNEST A. TROEGER, OF NEW YORK, N. Y., ASSIGNOR, BY MESNE ASSIGNMENTS, TO  
TRANS-LUX DAYLIGHT PICTURE SCREEN CORPORATION.

## TRANSLUCENT SCREEN FOR PROJECTION MACHINES.

Application filed August 21, 1925. Serial No. 51,578.

This invention relates to screens upon which pictures are projected, and more particularly to a translucent screen which is adapted to be interposed between a camera 5 and the audience.

It has been proposed to make translucent screens out of various substances including layers of different materials consisting of raw materials and heterogeneous compounds 10 and mixtures, but these screens have all had some undesirable properties such as fragility, lack of self-sustaining strength, liability to decomposition by the action of moisture, and absence of proper translucent characteristics required for correct reproduction of an 15 image and softness of light passing therethrough. An attempt to improve any one of these characteristics in translucent screens heretofore produced results in seriously affecting another characteristic and in most 20 cases the translucent efficiency of the screen. It is, therefore, among the purposes of my invention to produce a translucent screen having such fineness and smoothness of texture or grain and clearness of color as to 25 very distinctly bring out and show the image, either in natural colors or in black and white, without causing any fatigue to the eyes of an observer, and at the same time 30 obtaining a screen in which the undesirable characteristics recited above are obviated.

Another object is to produce a screen 35 which will be impervious to the deleterious effects of moisture and have sufficient firmness and toughness to withstand sagging while in use and yet be so flexible as to permit being rolled as a curtain and for storage purposes when not in use without in any way detracting from its translucent efficiency.

Other objects and uses of the invention will appear hereinafter in the description and claims.

As illustrated in the drawing, the translucent screen is designed to be placed between a cinematograph or any projecting 45 machine and the audience and the rays of light passing from the projection machine and through the film are directed upon the 50 screen from the rear. It is at once evident that this screen must have excellent translucent properties as well as to be able to soften the light which passes therethrough

and toward the audience. In obtaining such a screen, care must also be exercised in gaining mechanical properties which will suffice to withstand at least ordinary use and exposure without detracting from the high character of translucency desired, and I have discovered that a composition including pure 55 gum rubber, properly treated and tinted, is admirably adapted to fulfill both light and mechanical requirements.

In preparing the composition for my screen it is necessary to use about ninety- 60 seven per cent of pure gum rubber with about one per cent of oxide of zinc and about two per cent of an aniline dye of a selected color. The proportions of the various ingredients may be varied to some extent without varying the character of the actual product, but I have obtained a satisfactory screen 65 with the proportions set forth.

These ingredients must be kneaded together very thoroughly, in a manner well 70 known in the art, under proper heat conditions, until a homogeneous dough-like product of uniform texture and tint results. This product is then rolled into sheets by a calendering machine which may be designed to 75 leave one side smooth and the other side slightly roughened, as, for example, by the 80 impressions resulting from having one of the calendering rolls covered with fabric. This roughened surface is positioned, when 85 the screen is ready for use, toward the audience and it aids in the light diffusion. Both sides, however, could be left smooth 90 since the character of the screen itself tends to diffuse the light and thereby prevent glare. After the sheets are rolled, they are 95 steam-cured and are then ready for use.

In order to obtain good results I have found that the thickness of the sheets should preferably be about fifteen gauge, but thicknesses ranging from ten gauge to thirty gauge give good results under different conditions.

As well as serving as a necessary medium in the steam-curing process, the zinc oxide is 100 a useful factor which aids in making the rubber screen adaptable to make the images stand out and be clearly legible. It also serves, together with the selected aniline dye, to give a desired tint to the screen and hence 105 to the appearance of the image. The tinted

screen serves to filter out the harsh colors emitting from the lamp in the projecting machine, and I have had excellent results in producing a soft and restful light effect by the use of a blue aniline dye.

A sheet of rubber produced by the steps hereinbefore stated is tough and flexible and slightly elastic, thereby having inherent mechanical properties which render it suitable for curtain and screen purposes. It is not liable to sag and wrinkle or become distorted under varying climatic conditions and its elasticity enables it to be kept taut and smooth at all times. Its excellent translucent properties are dependent upon the prepared material itself, and its mechanical characteristics enable it to be manufactured and used at thicknesses which have not been heretofore attainable.

Changes in duration and manner of treatment are contemplated within the scope of the appended claims, and I do not wish to be limited to the exact proportions of ingredients specified.

What I claim is—

1. A projection screen comprising a sheet of translucent cured rubber material.
2. A projection screen comprising a sheet of translucent cured rubber having a diffuser incorporated therein.
3. A projection screen comprising a sheet of translucent cured elastic rubber material.
4. A projection screen formed of a sheet of translucent rubber material containing a small percentage of zinc oxide.
5. A projection screen comprising a sheet of translucent cured rubber as its principal constituent.
6. A projection screen formed of a sheet of pure gum rubber and also containing a small percentage of zinc oxide.
7. A projection screen formed of a sheet of pure gum rubber and also containing a

small percentage of zinc oxide and a coloring dye.

8. A projection screen formed of a sheet of translucent pure gum rubber rolled and steam-cured.

9. A projection screen formed of a sheet of material containing approximately 97% pure gum rubber, approximately 1% zinc oxide, and approximately 2% of coloring dye.

10. A projection screen formed of a sheet of material containing approximately 1% zinc oxide and a preponderance of pure gum rubber.

11. A projection screen formed of a sheet of material containing approximately 97% pure gum rubber, approximately 1% zinc oxide, and approximately 2% coloring dye, the sheet being rolled and steam-cured.

12. A projection screen formed of a sheet of material containing approximately 1% zinc oxide and a preponderance of pure gum rubber, the sheet being rolled and steam-cured.

13. A projection screen comprising a sheet of translucent cured rubber material of a thickness between ten gauge and thirty gauge.

14. A projection screen comprising a sheet of translucent cured rubber material of a thickness of approximately fifteen gauge.

15. A translucent projection screen comprising a cured rubber sheet having incorporated therein a diffuser.

16. A projection screen comprising a sheet of translucent cured rubber material of a thickness between ten gauge and thirty gauge, and having incorporated therein a diffuser.

In testimony whereof I hereto affix my signature.

ERNEST A. TROEGER.